

1

2,905,640

**PETROLEUM LUBRICANT STABILIZED AGAINST HYDROCARBON-METABOLIZING MICRO-ORGANISMS**

Edward B. Hodge, Terre Haute, Ind., assignor to Commercial Solvents Corporation, Terre Haute, Ind., a corporation of Maryland

No Drawing. Application August 1, 1957  
Serial No. 675,528

3 Claims. (Cl. 252—51.5)

My invention relates to a stabilized petroleum lubricant and more particularly to a process for the production of stabilized petroleum lubricants containing 5-amino-2,2,5-trimethyl-3-aza-1-hexanol as the active stabilizing agent.

It is well known that organisms from the group consisting of *Corynebacterium*, *Achromobacter*, *Nocardia*, *Pseudomonas*, *Mycobacterium*, etc., metabolize petroleum hydrocarbons and fatty acids and thereby produce undesirable oxidation products.

The petroleum industry has long been interested in the stabilization of various petroleum products such as cutting oils, hydraulic oils, hydraulic fluids, etc., against break-down by bacteria which metabolize the hydrocarbons with the concurrent formation of deleterious metabolites.

Many compounds have been used as stabilization agents in lubricants, but very few have been found to be commercially successful due to the fact that the compounds are unstable, or are not active against a wide variety of microorganisms.

I have now discovered that 5-amino-2,2,5-trimethyl-3-aza-1-hexanol is very active against petroleum metabolizing microorganisms. This compound can be easily prepared in good yields by the method set out in U.S. Patent 2,393,825. I have found that in some instances I can obtain total inhibition of bacterial growth in petroleum lubricants at concentrations as low as 0.005%. I prefer to include at least 0.0075% in most petroleum formulations. However, I can employ amounts up to 10.0% of the active agent when the latter is soluble to this extent in the particular petroleum hydrocarbon compositions.

I have found that 2-amino-2,2,5-trimethyl-3-aza-1-hexanol is an effective bacteriostatic agent in petroleum containing lubricants such as cutting oils, penetrating oils, grinding lubricants, iron tinning lubricants, core oils, hydraulic fluids, etc.

The following examples set out lubricating compositions in which 5-amino-2,2,5-trimethyl-3-aza-1-hexanol acts as an effective bacteriostatic agent. It is not intended that my invention be limited to the compositions, portions, or lubricants set out below, but rather I intend for all the equivalents and variations obvious to those skilled in the art to be included within the scope of this specification and the attached claims.

*Example I*

A water soluble cutting oil containing 2-amino-2,2,5-trimethyl-3-aza-1-hexanol was tested for activity against petroleum metabolizing organisms by preparing a composition having the formula:

|                             | Percent by weight |
|-----------------------------|-------------------|
| Light mineral oil           | 85                |
| Oleic acid                  | 10                |
| 2-amino-2-methyl-1-propanol | 5                 |

2

Two equal proportions of this formulation were prepared and enough 5-amino-2,2,5-trimethyl-3-aza-1-hexanol was added to one portion to create a 750γ/ml. concentration. Both portions were then diluted 1:10 with north gelatin agar (Difco) and streaked with an 18 hour agar slant culture of the representative organism *Pseudomonas aeruginosa*. The control and stabilized compositions were then incubated for 18 hours at 35° C. and the growth was recorded. Complete inhibition was exhibited by the stabilized composition while a growth of 4+ was noted on the control composition.

*Example II*

15 A steam cylinder oil composition having the following formula:

|                                         |          |
|-----------------------------------------|----------|
| S.A.E. lubricating oil                  | 90%      |
| Oleic acid                              | 10%      |
| 5-amino-2,2,5-trimethyl-3-aza-1-hexanol | 750γ/ml. |

20 was diluted and tested by the method of Example I. The stabilized composition was found to exhibit no growth while the control composition exhibited a bacterial growth of 4+.

*Example III*

25 A core oil having the following composition:

|                                       |          |
|---------------------------------------|----------|
| Crude tall oil                        | 25%      |
| Fuel oil                              | 35%      |
| Tall oil ester (glycol or glycerol)   | 40%      |
| 5-amino-2,2,5-trimethyl-3-aza-hexanol | 750γ/ml. |

30 was diluted and tested by the method of Example I. The stabilized portion was found to exhibit no bacterial growth while the control composition exhibited a growth of 4+.

*Example IV*

35 A cutting oil and grinding lubricant having the following composition:

|                                         |          |
|-----------------------------------------|----------|
| Tallow                                  | 65%      |
| Paraffin wax                            | 29%      |
| Beeswax                                 | 1%       |
| Citric acid                             | 1.3%     |
| Oxalic acid                             | 1.3%     |
| Potassium citrate                       | 1.3%     |
| 45 Urea                                 | 0.4%     |
| 5-amino-2,2,5-trimethyl-3-aza-1-hexanol | 750γ/ml. |

40 was diluted and tested by the method of Example I. No bacterial growth was found on the stabilized composition while the control composition exhibited a bacterial growth of 4+.

45 Now having described my invention, what I claim is:

1. A petroleum lubricant stabilized against hydrocarbon-metabolizing micro-organisms containing a small but sufficient amount to inhibit said petroleum metabolizing 50 micro-organisms of 5-amino-2,2,5-trimethyl-3-aza-1-hexanol.

2. An aliphatic petroleum hydrocarbon lubricant stabilized against hydrocarbon-metabolizing micro-organisms containing from 0.005% to 10.0% by weight of 5-amino-2,2,5-trimethyl-3-aza-1-hexanol.

3. An aliphatic petroleum hydrocarbon lubricant stabilized against hydrocarbon-metabolizing micro-organisms containing from 0.0075% to 10.0% by weight of 5-amino-2,2,5-trimethyl-3-aza-1-hexanol.

**References Cited in the file of this patent**

UNITED STATES PATENTS

2,393,825 Senkus Jan. 29, 1946